

1,370,234.

G. W. STEWART.

SHEET PACKING.

APPLICATION FILED SEPT. 30, 1919.

Patented Mar. 1, 1921

*Fig. 1.*



*Fig. 2.*



Inventor

George W. Stewart  
By his Attorney  
L. George Stewart

# UNITED STATES PATENT OFFICE.

GEORGE W. STEWART, OF WEEHAWKEN, NEW JERSEY.

## SHEET-PACKING.

1,370,234.

Specification of Letters Patent.

Patented Mar. 1, 1921.

Application filed September 30, 1919. Serial No. 327,362.

*To all whom it may concern:*

Be it known that I, GEORGE W. STEWART, residing at Weehawken, in the county of Hudson and State of New Jersey, have invented certain new and useful Improvements in Sheet-Packings, of which the following is a specification.

This invention relates to sheet packing such as is commonly used for the making of gaskets and the like.

An object of the invention is to provide a sheet packing which is more substantial and durable in use than heretofore.

A more detailed object is to provide a packing consisting of a plurality of layers of different materials all compressed into sheet form and the whole being of such composition and consistency as to be capable of serving its intended purpose for greatly prolonged periods without likelihood of disintegration.

Other objects and aims of the invention, more or less specific than those referred to above, will be in part obvious and in part pointed out in the course of the following description of the elements, combinations, arrangements of parts and applications of principles, constituting the invention; and the scope of protection contemplated will be indicated in the appended claims.

In the accompanying drawings which are to be taken as a part of this specification, and in which I have shown merely a preferred form of embodiment of the invention:—

Figure 1 is a perspective view of a portion of sheet packing constructed in accordance with this invention, certain of the layers of materials comprising the packing being shown spread apart for better disclosing the construction of the packing, and

Fig. 2 is an enlarged fragmentary sectional view through a portion of the packing shown in Fig. 1.

Referring to the drawings for describing in detail the structure which is illustrated therein, the reference character L indicates one of the main layers of material employed. The reference character G indicates another similar layer and the reference character H indicates a layer of wire gauze or the like which is placed between the layers L and G.

The layers L and G preferably consist of a composition of asbestos fiber and rubber properly compressed as is well known in connection with the manufacture of ordinary

compressed asbestos sheet packing. In the manufacture of these two layers the inner surfaces thereof, that is, the surfaces which are to lie adjacent the gauze H, are preferably left rough and unfinished so that the fiber of the asbestos material projects freely therefrom throughout the surface extent, as is indicated at 1.

Prior to applying the layers L and G to the opposite sides of the gauze H the fibrous surfaces of the layers L and G are each coated with a layer, as 2, of cementitious material consisting preferably of a composition of shellac and red lead. This coating is so applied that it adheres to and mixes with the protruding fibers forming the surfaces of the layers L and G. In this way the coating is made to become substantially an integral portion of the layers L and G, separation being practically impossible.

When the layers L and G, thus coated, are brought together under pressure against the opposite surfaces of the layer of gauze H, the material forming the coatings is made to squeeze through the openings in the gauze and to adhere firmly the coating of one layer to the coating of the other layer. The pressure applied upon the outer surface of the layers is preferably such as to cause the coatings to squeeze closely and firmly about all parts of the gauze so that a good mechanical bond is effected.

If desired the gauze itself may be coated or painted over, as at 3, with the cementitious material before it is placed between the layers L and G. In this way the cementitious material of the coatings 2 may be made to more easily and intimately fix themselves upon the gauze as well as upon each other.

If desired, also the outer surfaces of the main layers L and G may be coated over, as at 4, with a suitable waterproofing paint, or the like, such as shellac.

It has been noted that gaskets formed from the usual compressed asbestos sheet packing are susceptible to early deterioration when subjected to the action of moisture and the like, and in this connection it should be pointed out that in the packing above described, the composition of shellac and red lead so placed as to combine with the rubber and asbestos layers serves as a very effective moisture excluding agent, while at the same time not interfering with the desirable resiliency of the outermost portions

of the asbestos and rubber layers. The exclusion of moisture from within the body of the packing will thus very materially delay the action of disintegrating forces and will 5 enable a gasket, formed of the packing, to maintain its original shape and effectiveness for long periods of time.

The wire gauze is of equal importance in prolonging the life of the gasket since it 10 will serve to hold the gasket against actual disintegration long after the process of dissolution and disintegration has begun.

In addition to its moisture excluding qualities the coatings 2 are equally valuable 15 in performing their office of cementing together the main layers of rubber and asbestos upon the interposed gauze.

The outer coatings 4 of moisture proofing material not only serve to increase the 20 resistance of the packing to the effects of moisture but, especially when shellac is employed for these coatings, they also serve as a cement to cement the gaskets to the machine parts between which the gasket is 25 placed in use, thus further delaying actual disintegration of the gasket.

The coating 3, which is applied to the wire gauze prior to application of the gauze between the layers of the packing, is particularly 30 advantageous since it effectively closes all of the interstices of the gauze and prevents likelihood of the formation of voids or minute moisture carrying passages along the wires of the gauze when 35 the gauze has been placed between the layers.

As many changes could be made in this construction without departing from the scope of the invention as defined in the following claims, it is intended that all matter 40 contained in the above description or shown in the accompanying drawings, shall be interpreted as illustrative only and not in a limiting sense.

Having thus described my invention, 45 what I claim as new and desire to secure by Letters Patent is:—

1. A packing of the class described comprising a pair of layers of resilient fibrous material, a body of material interposed between 50 said layers serving to bind said layers together and being of a moisture resisting character and coatings of cement material covering the outer surfaces of said layers for the purpose described.

55 2. A packing of the class described comprising a pair of layers of resilient fibrous material each of said layers having a coating of moisture resisting cementitious ma-

terial covering one of its surfaces, a layer of wire gauze interposed between said first 60 layers and said first layers being pressed against opposite sides of said wire gauze so that said coatings engage together and adhere to each other and to said wire gauze.

3. A packing of the class described comprising a pair of layers of resilient fibrous material, each of said layers having a coating of moisture resisting cementitious material covering one of its surfaces, a layer of wire gauze interposed between said first 70 layers, a coating of cementitious material covering the wires of said gauze, and said first layers being pressed against opposite sides of said wire gauze so that the coatings of said first layers engage together and adhere to each other and to the coating of 75 said wire gauze.

4. A packing of the class described comprising a pair of layers each consisting of a composition of asbestos fiber and rubber, 80 each of said layers having a coating of moisture resisting cementitious material covering one of its surfaces consisting of a composition of red lead and shellac, a layer of wire gauze interposed between said first 85 layers, and said first layers being pressed against opposite sides of said wire gauze so that said coatings engage together and adhere to each other and to said wire gauze.

5. A packing of the class described comprising a pair of layers each layer being composed of a compressed composition of asbestos fiber and rubber, a layer of wire gauze interposed between said first layers, and a body of cementitious material also 95 interposed between said first layers having said wire gauze embedded therein holding all of said layers together substantially throughout their extent.

6. A packing of the class described comprising a pair of layers of resilient fibrous material, moisture resisting material covering one surface of each of said layers, a layer of wire gauze interposed between said first layers, said first layers being positioned so that the surfaces of said moisture resisting material engage the opposite sides of said wire gauze, and means holding all of said layers together substantially throughout their extent.

In testimony whereof I affix my signature in the presence of two witnesses.

GEORGE W. STEWART.

Witnesses:

L. GESSFORD HANDY,  
S. J. AUMILLER.